

## UNITED STATES PATENT OFFICE

BRUNO WENDT, OF DESSAU IN ANHALT, AND HANS BINCER, OF DESSAU-ZIEBIGK IN ANHALT, GERMANY, ASSIGNORS TO AGFA ANSCO CORPORATION, OF BINGHAMTON, NEW YORK, A CORPORATION OF NEW YORK

## FIXING BLEACHING-OUT PICTURES

No Drawing. Application filed April 25, 1930, Serial No. 447,420, and in Germany May 11, 1929.

Our present invention relates to a process of fixing photographic pictures and more particularly to a process of fixing such pictures obtained according to the bleaching-out method on a layer containing a basic dye sensitized to the action of light by the presence of a sensitizer as, for instance, a derivative of thiourea, such as allylthiourea or the homologues or substitution products thereof.

10 In the known bleaching-out process the difficulty exists that the freshly printed pictures retain their sensitiveness to light and fade when exposed to light. The sensitiveness to light of such pictures can only be diminished by removing the sensitizer from the picture. This operation has, however, been difficult since the solvents for the sensitizer also attack the dyes constituting the picture.

20 According to this invention, for fixing such bleaching-out layers sulfurous acid is used with good result. It acts upon the derivative of thiourea serving as sensitizer without exerting any injurious influence on the dye.

25 The sulfurous acid may be used either in aqueous solution or dissolved in an organic solvent. The solvent selected for this purpose must be one which does not act upon the binding agent in the layer to be fixed in each of 30 bleaching out dyes constituting the picture case. It is, however, particularly advantageous to fix by means of gaseous sulfur dioxide.

According to the nature of the binding 35 agent of the layer, the product of the action of sulfurous acid on the sensitizer remains in the layer or segregates on its surface. In the first case, the product may either be left in the layer or be removed by means of a swelling agent which does not attack the dye, for instance, a mixture of benzene and alcohol; in the second case, the surface is purified in a mechanical way or by means of an indifferent liquid, for instance, benzene.

45 The following example serves to illustrate the invention:

A picture made by the bleaching-out process the binding agent of which consists of nitrocellulose and which contains diethyl- 50 allylthiourea as a sensitizer, is placed for

about 3 hours in a closed vessel on the bottom of which there is a dish charged with an aqueous solution of sodium bisulfite. On the layer a decomposition product of the sensitizer, which is of unknown constitution segregates in the form of oily drops which are removed by means of a piece of fabric moistened with benzene. 55

The invention is not limited to the foregoing example or to the specific details given 60 therein. Thus, for instance, instead of an aqueous solution of sodium bisulfite a solution of sulfurous acid in a suitable solvent evolving gaseous sulfur dioxide may be used. Or, the unfixed picture may be treated in a 65 bath containing in the case of nitrocellulose used as a binding agent for the dye a mixture of benzene and methyl alcohol in the ratio 4:1 and sulfurous acid in a quantity up to saturation. Thus, the fixing process is 70 finished in about 20 minutes.

In the same manner, other layers containing other sensitizers of the group comprising derivatives of thiourea, may be fixed.

What we claim is:—

1. The process of fixing bleaching-out 75 layers containing a derivative of thiourea as a sensitizer, which comprises acting upon said layer which sulfurous acid.

2. The process of fixing bleaching-out 80 layers containing a derivative of thiourea as a sensitizer, which comprises acting upon said layer with gaseous sulfur dioxide.

3. The process of fixing bleaching-out 85 layers containing allylthiourea as a sensitizer, which comprises acting upon said layer with sulfurous acid.

4. The process of fixing bleaching-out 90 layers containing allylthiourea as a sensitizer, which comprises acting upon said layer with gaseous sulfur dioxide.

In testimony whereof, we affix our signatures.

BRUNO WENDT.  
HANS BINCER.

95

10